

June 3, 1930.

F. S. McCULLOUGH

1,761,577

METHOD OF MANUFACTURING WIRE AND PORCELAIN ELEMENTS

Filed Jan. 5, 1926

Fig. 1



Fig. 2



Fig. 3



INVENTOR  
Frederick S. McCullough  
By Hynes, Stabbins & Pardee  
his attorneys.

## UNITED STATES PATENT OFFICE

FREDERICK S. McCULLOUGH, OF EDGEWOOD, PENNSYLVANIA

## METHOD OF MANUFACTURING WIRE AND PORCELAIN ELEMENTS

Application filed January 5, 1926. Serial No. 79,351.

This invention relates to a method of placing wires in porcelain or other refractory or ceramic material.

In certain types of electrical apparatus, it is customary to have a wire embedded in a refractory insulating material. Reference is made particularly to electric heaters of certain types, such as those used in confined spaces, as for instance, the heaters of cathodes of certain types of space discharge devices.

In heaters of this type, the best results are effected if the wire is in intimate contact with the refractory material. At the same time, the heater must be manufactured according to a process that will not destroy the frail and readily oxidizable heater wire. According to practices heretofore followed, the porcelain or refractory rod in which the wire is subsequently to be placed, is formed by a process of extrusion, after which the rods are fired and cut to length. The heater wire is then passed through the fired porcelain rod sections in holes originally formed in the material by the extrusion process.

According to the present invention it is proposed to extrude the porcelain, cut it to lengths after it has set, insert the heater wires, and then fire the porcelain, contracting it onto the wires, the firing taking place under conditions conducive to a maximum shrinkage, and without liability of oxidation of the heater wire.

The nature of the invention may be readily understood by reference to the accompanying drawings, wherein:

Figure 1 represents an elevation of a section of unfired porcelain before the passage of the heater wire therethrough, the figure showing the material somewhat larger than that commonly employed;

Figure 2 is a longitudinal section through the porcelain rod of Figure 1 with the heater wire in place; and

Figure 3 is a vertical section illustrating diagrammatically a manner of firing the assembled structure shown in Figure 2.

In the drawings, 2 represents a length of rod of porcelain or other refractory mate-

rial having parallel holes 3 and 4 extending longitudinally therethrough. This section of rod is cut from a length of such material formed by a process of extrusion after the porcelain has set and before it is fired. 55 A bowed or "hairpin" shaped wire 5 of suitable resistance is then passed through the holes 3 and 4, as shown in Figure 2. This wire may be of tungsten or other suitable material.

The heater element, as the porcelain with the wire passed therethrough may be termed, may then be enclosed in a suitable chamber and fired. In Figure 3 I have illustrated one manner of doing this wherein the heater 65 element is suspended within a silica or other refractory chamber 6 having an outlet connection 7 leading to a suitable vacuum pump, not shown. I have shown chamber 6 as being closed by a suitable plug 8. 70

After the chamber 6 has been evacuated, and while the vacuum is maintained therein, it is placed in a suitable heating furnace, designated 9 and the porcelain 2 is fired at a high temperature. The refractory material contracts onto the metal, so that the two are in more intimate contact than has heretofore been possible. At the same time, the temperature can be sufficiently high to effect a thorough burning of the refractory 80 material without damage to the heating wire, as oxidation does not occur.

After being heated at the desired temperature for a necessary period of time, the chamber may be removed from the furnace. 85

Heaters as thus produced are highly satisfactory. Assembly thereof is facilitated because when the wires are put through the porcelain, the holes 3 and 4 are fairly open.

Various detail changes may be made in the practice of the invention, and the invention is not restricted to the manufacture of the particular construction of heater shown, or to the use of any particular apparatus.

I claim as my invention:

1. A method of making refractory bodies with wires therethrough which consists in forming a length of refractory rod with a hole therethrough, allowing the refractory material to set, then passing a wire through 100

the hole, and firing the refractory rod with the wire therein under conditions which preclude oxidation of the wire.

2. A method of making refractory bodies with wires therethrough which consists in forming a length of unvitrified refractory rod with a hole therethrough, allowing the refractory material to set, then passing a wire through the hole in the unvitrified rod, and firing the refractory rod with the wire therein in a vacuum.

3. A method of making heater elements which consists in forming a rod of ceramic material having a hole therethrough, passing a wire through the hole, enclosing the assembled structure in a chamber, and heating the chamber to fire the ceramic material while maintaining a vacuum in the chamber.

4. A method of forming heaters which consists in forming a rod of unvitrified porcelain with a hole therethrough, allowing the porcelain to set, then passing a wire through the hole in the unvitrified rod, and contracting the porcelain onto the wire by firing the same under conditions precluding oxidation of the wire.

5. A method of forming heaters which consists in applying a mass of refractory substance to a wire and in intimate contact with the wire, then heating the resulting structure in a vacuum to bake the refractory into intimate contact with the wire and to remove the gas therefrom and prevent oxidation of the wire.

In testimony whereof I have hereunto set my hand.

FREDERICK S. McCULLOUGH.

#### CERTIFICATE OF CORRECTION.

Patent No. 1,761,577.

Granted June 3, 1930, to

FREDERICK S. McCULLOUGH.

It is hereby certified that error appears in the printed specification of the above numbered patent requiring correction as follows: Page 1, line 98, claim 1, before the word "refractory" insert the word unvitrified, and page 2, line 1, same claim, after the word "hole" insert the words in the unvitrified rod; same page, line 6, claim 2, strike out "unvitrified", and line 9, strike out "in the unvitrified rod"; and that the said Letters Patent should be read with these corrections therein that the same may conform to the record of the case in the Patent Office.

Signed and sealed this 13th day of January, A. D. 1931.

(Seal)

M. J. Moore,  
Acting Commissioner of Patents.

the hole, and firing the refractory rod with the wire therein under conditions which preclude oxidation of the wire.

2. A method of making refractory bodies with wires therethrough which consists in forming a length of unvitrified refractory rod with a hole therethrough, allowing the refractory material to set, then passing a wire through the hole in the unvitrified rod, and firing the refractory rod with the wire therein in a vacuum.

3. A method of making heater elements which consists in forming a rod of ceramic material having a hole therethrough, passing a wire through the hole, enclosing the assembled structure in a chamber, and heating the chamber to fire the ceramic material while maintaining a vacuum in the chamber.

4. A method of forming heaters which consists in forming a rod of unvitrified porcelain with a hole therethrough, allowing the porcelain to set, then passing a wire through the hole in the unvitrified rod, and contracting the porcelain onto the wire by firing the same under conditions precluding oxidation of the wire.

5. A method of forming heaters which consists in applying a mass of refractory substance to a wire and in intimate contact with the wire, then heating the resulting structure in a vacuum to bake the refractory into intimate contact with the wire and to remove the gas therefrom and prevent oxidation of the wire.

In testimony whereof I have hereunto set my hand.

FREDERICK S. McCULLOUGH.

#### CERTIFICATE OF CORRECTION.

Patent No. 1,761,577.

Granted June 3, 1930, to

FREDERICK S. McCULLOUGH.

It is hereby certified that error appears in the printed specification of the above numbered patent requiring correction as follows: Page 1, line 98, claim 1, before the word "refractory" insert the word unvitrified, and page 2, line 1, same claim, after the word "hole" insert the words in the unvitrified rod; same page, line 6, claim 2, strike out "unvitrified", and line 9, strike out "in the unvitrified rod"; and that the said Letters Patent should be read with these corrections therein that the same may conform to the record of the case in the Patent Office.

Signed and sealed this 13th day of January, A. D. 1931.

(Seal)

M. J. Moore,  
Acting Commissioner of Patents.